

# United States Patent Office

2,829,958

Patented Apr. 8, 1958

1

2,829,958

## EXPLOSIVE COMPOSITIONS

Samuel Henry Davidson, Largs, Scotland, and Thomas Balfour, Northrand, Union of South Africa, assignors to Imperial Chemical Industries Limited, London, England, a corporation of Great Britain

No Drawing. Application April 8, 1955  
Serial No. 500,268

Claims priority, application Great Britain April 26, 1954

5 Claims. (Cl. 52—7)

The present invention is concerned with new and improved ammonium nitrate explosive compositions of the kind which are safe for use in methane-air mixtures and which would be regarded as permitted or permissible for use in fiery coal-mines and more particularly to such compositions which are free from self-explosive organic materials and cartridges therefrom.

In the manufacture of such explosive compositions it is customary to include in the compositions self-explosive organic materials for example liquid explosive nitric esters or trinitro-aromatic compounds. These are not, however, always available and their manufacture involves a hazard additional to that associated with their mixing with the other ingredients of the final explosive composition. Furthermore the ammonium nitrate which is used is of the usual grit size and usually cannot be made to explode in cartridges of the general nature and size required to attain explosive compositions of the aforesaid kind. It is known, however, that a mixture of ammonium nitrate of grit size as ordinarily used in the manufacture of explosive compositions and aluminium powder can be caused to explode by means of a commercial detonator if the density of the mixture is suitably diminished by the inclusion therein of dry vegetable tissue. These vegetable tissue materials are specially effective in facilitating initiation when they are of intrinsically low bulk density, as for example balsa meal, cork dust and bagasse. However, explosive compositions of unusually low bulk density tend to become compacted during transport to a higher density with an adverse effect on their sensitiveness to initiation and propagation.

Although explosive compositions have been proposed for coal-mining which contain aluminium as an ingredient, as a result of increasingly stringent requirements in recent years in respect of freedom from danger in igniting methane, including for instance the introduction of official Gallery tests, no explosive composition containing aluminium as an ingredient has appeared for several years in the official list of explosives permitted for use in coal-mines for example by H. M. Home Office.

The object of the present invention is to provide explosive compositions for use in gassy or fiery mines which are free from self-explosive ingredients and have a satisfactory sensitiveness to initiation and capacity for propagation and bulk densities in a range high enough to be maintained during transport and a greater strength than any that have hitherto been found safe enough for use in gassy or fiery mines.

An explosive composition according to the invention comprises ammonium nitrate of particle size such that substantially all of it passes a 120 B. S. S. sieve, aluminium particles such that at least a part is paint-fine, vegetable tissue material, and at least one flame-quenching ingredient, and has a bulk density not less than 0.85 g./cc. and not greater than 1.1 g./cc. and is substantially oxygen balanced.

The power of the explosive compositions of the invention should preferably be less than 74% blasting gelatine,

2

If desired the explosive compositions of the invention may include organic ingredients for instance orthonitrotoluol.

Examples of flame-quenching ingredients are sodium chloride, sodium sulphate and china clay. If sodium chloride is the flame-quenching ingredient the quantity present should be at least 8% and preferably not more than 25%.

Preferably the ammonium nitrate in the compositions of the invention is of particle size such that not less than 60% passes a No. 240 B. S. S. sieve, not less than 80% passes a No. 170 B. S. S. sieve and substantially all, i. e., at least 98%, passes a No. 120 B. S. S. sieve. It is also preferred that the total amount of aluminium in the composition be not less than 1% and not more than 2.5% by weight and that not less than 0.5% and not more than 1% of the aluminium present based on the weight of the explosive composition be paint-fine aluminium. Furthermore a composition of the invention is satisfactorily oxygen balanced if its oxygen surplus or deficiency does not exceed 5 g. oxygen per 100 g. thereof.

Although ammonium nitrate of the aforesaid particle size enables explosive compositions of a greater degree of safety to be obtained than has hitherto been possible for explosive compositions of the same percentage composition and power, the improvement is still insufficient to enable the whole of the oxidisable content of the explosive composition to consist of aluminium. Again although the sensitising effect on ammonium nitrate of paint-fine aluminium is higher than that of granular aluminium the tendency of paint-fine aluminium to ignite methane-air mixtures is higher than that of granular aluminium and so the percentage of paint-fine aluminium that may be present in an explosive composition is even more severely limited than that of granular aluminium. Therefore, to achieve the desired sensitiveness to initiation and propagation of an explosive composition comprising ammonium nitrate in finely divided form and aluminium particles, at least part of which is paint-fine, it is essential to include at least a portion of the remainder of the oxidisable ingredients to make the composition oxygen balanced in the form of vegetable tissue material. Such material has the effect furthermore of reducing the density of the composition more than ordinary oxidisable organic compounds and it has been found that the bulk density of the explosive composition should not be higher than 1.1 g./cc. if satisfactory sensitiveness to initiation and propagation is to be achieved. On the other hand it is undesirable that the density should be lower than 0.85 g./cc. Examples of vegetable material suitable for use in the compositions of the invention are woodflour, which has a density of about 0.4 g./cc., or lower density materials as for instance balsa meal, ground cork or bagasse.

Ammonium nitrate as heretofore employed in explosives suitable for fiery or gassy coal-mines consists of crystal clusters or crystals of such size as to be substantially retained on a No. 170 B. S. S. sieve and is ineffective for the present invention. Thus at bulk densities between 0.85 and 1.1 g./cc. mixtures of the same percentage compositions containing such ammonium nitrate in place of the fine ammonium nitrate used in the compositions of the present invention are insensitive to commercial detonators and require the use of a booster the employment of which is not permitted in commercial coal-mining practice.

The invention is illustrated by compositions Nos. 1 to 5 and compared with compositions Nos. 6 to 9 not in accordance with the invention in the following table.

Nine explosive compositions are made by mixing together the ingredients as shown in the following table and are formed into cartridges of the sizes normally required

for coal-mining. These cartridges are tested in accordance with two Gallery tests. In accordance with one Gallery test it is not permissible to get a failure when five shots of 8 oz. each are fired from a mortar unstemmed in a Gallery containing 9% methane in a mixture of methane and air. In accordance with the second Gallery test five shots of 28 oz. stemmed with a 1 inch thick dry clay plug when fired into a Gallery containing 9% methane in a mixture of methane and air must not ignite the gas. The ammonium nitrate which is used in the nine explosive compositions is of particle size such that 80% by weight passes a No. 240 B. S. S. sieve and all of it passes a No. 120 B. S. S. sieve.

Ammonium nitrate of the usual commercial size, i. e. one wherein only 20% passes a No. 120 B. S. S. sieve and only 75% passes a No. 60 B. S. S. sieve when used to make the explosive compositions indicated in the following table produce explosive compositions of such reduced sensitiveness that they fail to fire when formed into cartridges of the ordinary commercial size for use in bore holes in mines when any commercial detonator is used.

passes a No. 240 B. S. S. sieve, not less than 80% thereof passes a No. 170 B. S. S. sieve and substantially all thereof passes a No. 120 B. S. S. sieve, from 1% to 5 2.5% of aluminum particles by weight of total composition wherein 0.5% to 1% of said particles by weight of total composition are of a pigment powder fineness, vegetable tissue material and at least one flame-quenching ingredient, and having a bulk density not less than 0.85 gram per cc. and not greater than 1.1 grams per cc. and being substantially oxygen balanced.

10 2. An explosive composition as claimed in claim 1 which includes organic ingredients.

15 3. An explosive composition as claimed in claim 2 wherein the organic ingredient is orthonitrotoluol.

4. An explosive composition as claimed in claim 1 wherein said flame-quenching ingredient is selected from the group consisting of sodium chloride, sodium sulphate and china clay.

20 5. An explosive composition as claimed in claim 4 wherein the quantity of sodium chloride is between 8% and 15%.

| Composition No. | Composition (parts) |                     |                   |               |         | Properties      |                                           |                   |                     | Gallery tests               |      |     |
|-----------------|---------------------|---------------------|-------------------|---------------|---------|-----------------|-------------------------------------------|-------------------|---------------------|-----------------------------|------|-----|
|                 | Ammonium nitrate    | Paint-fine aluminum | Granular aluminum | O-nitrotoluol | Bagasse | Sodium chloride | Oxygen surplus, g. O <sub>2</sub> /100 g. | Density, g./c. c. | Power (percent B/G) | Initiation by detonator No. | 1    | 2   |
| 1. 78           | 1                   | 1                   | 1                 | 5             | 5       | 10              | -1.2                                      | 1.10              | 71.8                | 6                           | 8-12 | >30 |
| 2. 82           | 1                   | 1                   | 1                 | 4             | 8       | 8               | +4.9                                      | 1.04              | 68.1                | 5                           | >12  | >30 |
| 3. 72           | 1                   | 1                   | 1                 | 1             | 10      | 18              | -3.5                                      | 0.86              | 63.0                | 4                           | >12  | >30 |
| 4. 70           | 1                   | 1                   | 1                 | 4             | 8       | 25              | 0                                         | 0.85              | 58.9                | 3                           | >12  | >30 |
| 5. 62           | 1                   | 1                   | 1                 | 5             | 4       | 6               | -5.0                                      | 0.93              | 51.2                | 5                           | >12  | >30 |
| 6. 83           | 1                   | 1                   | 1                 | 4             | 8       | -----           | -0.1                                      | 0.94              | 74.5                | 6                           | <8   | <28 |
| 7. 87           | 1                   | 1                   | 1                 | 5             | 8       | -----           | +2.0                                      | 0.85              | 80.3                | 4                           | <8   | <28 |
| 8. 89           | 1                   | 1                   | 1                 | 6             | 4       | 25              | +2.1                                      | 1.02              | 82.0                | 5                           | <8   | <28 |
| 9. 62           | 1                   | 1                   | 1                 | 4             | 8       | 25              | -5.5                                      | 0.92              | 51.8                | 8                           | >12  | >30 |

From the table it will be seen that compositions Nos. 1 to 5 and 9 pass both Gallery tests but composition No. 9 which is not within the invention as it has no paint-fine aluminium, is unsatisfactory because its sensitiveness is so low that a No. 8 detonator is required for its initiation.

There is no correlation between the power of any one of said explosive compositions and its sensitiveness. To 45 be satisfactory as a blasting explosive, however, it must be capable of initiation by a No. 6 or weaker detonator.

What we claim is:

1. An explosive composition having a power less than 50 74% blasting gelatine and comprising ammonium nitrate of particle size such that not less than 60% thereof

#### References Cited in the file of this patent

#### UNITED STATES PATENTS

- |    |           |           |               |
|----|-----------|-----------|---------------|
| 40 | 1,891,500 | Burrows   | Dec. 20, 1932 |
|    | 1,979,681 | Fox       | Nov. 6, 1934  |
|    | 2,398,071 | Barab     | Apr. 9, 1946  |
|    | 2,409,919 | Whetstone | Oct. 22, 1946 |
|    | 2,613,146 | Lowe      | Oct. 7, 1952  |

#### FOREIGN PATENTS

- |         |               |       |               |
|---------|---------------|-------|---------------|
| 649,473 | Great Britain | ----- | Jan. 24, 1951 |
|---------|---------------|-------|---------------|

#### OTHER REFERENCES

- |                                                               |       |       |
|---------------------------------------------------------------|-------|-------|
| Serial No. 393,137, Baron (A. P. C.) published June 15, 1943. | ----- | ----- |
|---------------------------------------------------------------|-------|-------|